

## UNITED STATES PATENT OFFICE

JOSEPH KENT SMITH, OF DETROIT, MICHIGAN, ASSIGNOR TO BERYLLIUM DEVELOPMENT CORPORATION, OF NEW YORK, N. Y., A CORPORATION OF DELAWARE

## BERYLLIUM ALUMINUM ALLOY

No Drawing. Application filed December 22, 1931. Serial No. 582,653.

This invention relates to alloys characterized by extreme lightness and great strength, having metallic beryllium as the predominating component of the alloy.

5 Inasmuch as elementary beryllium in unalloyed form tends to great brittleness, and therefore does not lend itself readily to rolling, forging, or those other mechanical operations necessary to bring metals into readily 10 usable forms, especially those forms used where extreme lightness is required, it has been found necessary to alloy beryllium with smaller quantities of aluminum so as to obtain an ultra-light metallic material possessing 15 those characteristics which will permit of the mechanical operations cited. The proportions of aluminum added to the beryllium will vary in quantity with the requirements of the situation, the lower the quantity of 20 aluminum added, the lighter the resulting alloy, but the greater the difficulties of mechanical manipulation. When the aluminum content of the alloy is as little as ten percent of the total, great precautions are 25 necessary in rolling or forging the alloy, while the alloy with thirty percent of aluminum, with a specific gravity of approximately 2.0, lends itself quite readily to all the usual mechanical operations. Alloys of 30 about equal parts of beryllium and aluminum are still easier to work, but they lack the greater strength and superior lightness of the alloys lower in aluminum. The alloy approximating seventy percent beryllium 35 and thirty percent aluminum represents best current practice in this series, presenting a nice balance between the various factors involved.

However, the simple binary beryllium-aluminum alloys, despite their greater strength as compared with pure aluminum, leave still something to be desired in the matter of strength, machinability, etc. I have found, in my invention, that by adding, 45 to any of the beryllium-aluminum alloy series in which beryllium predominates—from about 55% to about 70% with aluminum from about 25% to about 40%—small quantities of manganese and vanadium, with or without 50 simultaneous additions of small quantities

of molybdenum, significant increases in strength, machinability, etc. can be effected, without any material increase in the specific gravity of the alloy. The "heavy" metals mentioned as addition agents should never 55 exceed five percent of the total weight of the alloy, and, in the preferred compositions, these metals do not exceed two percent of the total.

If desired, such alloys can be made by the 60 addition of the requisite quantities of the free heavy metals to a molten beryllium-aluminum alloy. A better method consists in melting the beryllium and aluminum together, employing as a flux a mixture of the 65 chlorides and fluorides of calcium with some cryolite. To this the vanadium (and, if desired, the molybdenum) is added in the form of compounds readily reducible in the circumstances, like calcium vanadate (and 70 calcium molybdate). Under the conditions, elementary vanadium (and molybdenum) is formed by reduction and enters into the alloy. The manganese is added by means of a cleansing alloy, comprising aluminum, 75 magnesium and manganese. The magnesium almost all boils out readily, while the manganese and aluminum unite with the primary alloy, resulting in the final multi-constituent alloy. 80

As compared with the simple binary beryllium-aluminum alloy of seventy percent beryllium content, a similar alloy containing about one-half percent each of vanadium, molybdenum and manganese is 85 more readily workable, flows better, casts better, has greater strength and resistance to corrosion, and is more readily flexed without cracking. In sheet form, say from fifteen to twenty thousandths of an inch in thickness, a strength of one hundred thousand to one hundred and ten thousand pounds to the square inch is obtained. In such sheet form, the alloy is particularly useful for airplane wings and fuselage parts, or wherever else the combination of ultra-lightness, strength and bendability without breaking is essential. 95

The presence of the heavy metals hardens the aluminum eutectic, giving the multi- 100

constituent alloy a relatively low coefficient of friction; the alloy is therefore useful for piston rings, pistons, and similar moving parts involving frictional effects.

5 In cast form, alloys covered by this invention have tensile strengths ranging from thirty thousand to fifty thousand pounds per square inch.

The percentages are by weight.  
10 I claim:

1. A beryllium-aluminum alloy of approximately the following composition: beryllium from 55% to 70%, aluminum from 25% to 40%, and manganese molybdenum 15 and vanadium from about 1/2% to 2 1/2% each.

2. A beryllium-aluminum alloy of approximately the following composition: beryllium from 55% to 70%, aluminum 20 from 25% to 40%, and manganese, vanadium and molybdenum from about 1/2% to 2 1/2% each but not materially in excess of 5% in the aggregate.

In testimony whereof I have hereunto  
25 signed my name.

JOSEPH KENT SMITH.

30

35

40

45

50

55

60

65